

# UNITED STATES PATENT OFFICE.

ADOLF KERTESZ, OF MAINKUR, GERMANY.

## PROCESS OF PREPARING CLOTH FOR TESTING ITS RESISTANCE TO WEARING.

1,116,077.

Specification of Letters Patent.

Patented Nov. 3, 1914.

No Drawing.

Application filed March 14, 1914. Serial No. 824,692.

To all whom it may concern:

Be it known that I, ADOLF KERTESZ, a subject of the Kingdom of Hungary, and a resident of Bismarckstrasse 5, Mainkur, Germany, have invented certain new and useful Improvements in Processes of Preparing Cloth for Testing Its Resistance to Wearing.

Heretofore it has been the general practice to test the quality and strength of cloth on the dynamometer by determining the elasticity and the resistance to tearing. It has however been observed that in the great majority of cases the values thus obtained do not yield a correct measurement of the resistance to wearing, and the quality of cloth could not be determined but by prolonged wearing-tests, as it is indeed the general practice of the military authorities.

In order to obtain a better mode of measurement it has been tried to test the cloth by scraping and rubbing; but the values thus obtained were so inexact and incorrect that no conclusions could be drawn therefrom. The royal office for the testing of materials at Lichtenfelde (see Lehne's *Färbereitung* 1911, page 118) remarked very inadequately that it is not possible to test in this way.

It has now been discovered that an excellent measure of the resistance of cloth to wear and tear is obtained by treating it previous to testing in such a way that the interior parts and the surface become perfectly uniform, and only subsequently testing the cloth on a scraping, rubbing, or other kind of grinding or beating machine.

The production of perfect evenness of the interior and the surface of the cloth is the significant point of the invention and may be attained by the following means: (a) the samples are first thoroughly wetted and then dried and evenly pressed; (b) the samples are boiled in water alone or in water containing slight quantities of alkalis, acids, glycerin, sulfoleates or similar very gently acting substances, and subsequently dried and possibly pressed; (c) the samples are treated with alcoholic or ethereal liquids or hydrocarbons and dried; (d) the samples are evenly raised by mechanical means and then pressed.

The treatments may be modified according to requirements or one may be combined with another. Very good results are obtained *e. g.* by treating one hour with alco-

hol, then  $\frac{1}{2}$  hour at 80-90° C. in water and after drying and uniform pressing finally testing on a scraping machine. Thus the various kinds of military cloth in use in Germany have given the following comparative values on an average on being subjected twice to comparative tests.

|                                          | Dynamometer.     |             | Scraping machine after preparatory treatment. | 65 |
|------------------------------------------|------------------|-------------|-----------------------------------------------|----|
|                                          | Breaking strain. | Elasticity. |                                               |    |
|                                          |                  |             |                                               | 70 |
| Dark blue cloth for coats.....           | 67.3             | 11.4        | 93                                            |    |
| Medium blue cloth for coats.....         | 66               | 11          | 100                                           |    |
| Blue mixed shade cloth for trousers..... | 69               | 11.8        | 118                                           |    |
| Fieldgray cloth for coats.....           | 67.6             | 12.2        | 84                                            |    |
| Fieldgray cloth for trousers.....        | 72.3             | 13.4        | 90                                            |    |

The experiences gathered allow of the conclusion that the values obtained by the new method are more reliable than the former, and a further proof is adduced by treating the cloth with substances which undoubtedly deteriorate the wool, *e. g.* soda or chlorid of lime and subsequently testing it comparatively on a dynamometer and on a scraping machine after the indicated preparatory treatment.

Fieldgray military cloth was treated as described below and then tested.

|                                                                                                                                                              | Testing on the dynamometer. |             | Testing on the scraping machine after the treatment indicated above. | 90  |
|--------------------------------------------------------------------------------------------------------------------------------------------------------------|-----------------------------|-------------|----------------------------------------------------------------------|-----|
|                                                                                                                                                              | Breaking strain.            | Elasticity. |                                                                      |     |
|                                                                                                                                                              |                             |             |                                                                      | 95  |
| (a) Fieldgray cloth.....                                                                                                                                     | 66.8                        | 11.9        | 100                                                                  |     |
| (b) Cloth (a) boiled one hour with 40 times its weight of water to which 1/2 gram soda ash per liter had been added.....                                     | 67.9                        | 10.2        | 94                                                                   | 100 |
| (c) Like (b) with 1 gram soda ash per liter.....                                                                                                             | 61.8                        | 9.2         | 67                                                                   |     |
| (d) Cloth (a) treated with chlorid of lime 1/5° Baume by first acidulating the cloth, then chlorinating, acidulating, and finally rinsing until neutral..... | 80.1                        | 10.6        | 76                                                                   |     |
| (e) Like (d) with chlorid of lime 2/5° Baume.....                                                                                                            | 77.6                        | 10.3        | 64                                                                   | 105 |

It is to be noticed from these figures that the breaking strength and elasticity as shown by the dynamometer is but slightly diminished whereas the new method of testing shows a gradual decrease up to 33

per cent. It is further demonstrated that the values of breaking strength are considerably increased by the treatment with chlorid of lime and the elasticity is but slightly diminished whereas the new method of testing indicates deteriorations of 34-36 per cent.

That the values obtained by the new method are more correct may be directly deduced from the fact that the treatment with soda is detrimental to the wool and that chlorinated wool, so-called silk-wool has been found to be much less durable to wearing than non-chlorinated wool.

Having now particularly described and ascertained the nature of the said invention and in what manner the same is to be performed, I declare that what I claim is:

1. The process of preparing cloth for testing its resistance to wearing, consisting in

subjecting the cloth to wetting and pressing, boiling, treating with alcoholic liquids, and raising and pressing.

2. The process of preparing cloth for testing its resistance to wearing, consisting in 25 subjecting the cloth to wetting and pressing, boiling, treating with hydrocarbons, and raising and pressing.

3. The process of preparing cloth for testing its resistance to wearing, consisting in 30 subjecting the cloth to wetting and pressing, boiling, treating with ethereal liquids, and raising and pressing.

In witness whereof I have hereunto signed my name this 26th day of February, 1914, 35 in the presence of two subscribing witnesses.

ADOLF KERTESZ.

Witnesses:

JEAN GRUND,  
CARL GRUND.

Copies of this patent may be obtained for five cents each, by addressing the "Commissioner of Patents, Washington, D. C."